



neutralize both acid groups, at about 50° C. in an alcoholic solution and thereafter recovering the amine salt from the alcoholic solution.

## EXAMPLE V

Following the procedure of Example IV, the tert-octadecylamine salt of decylmercaptomethylphosphonic acid was prepared using tert-octadecylamine, available commercially under the trade name of Primeme JM-R, instead of di-2-ethylhexylamine.

The following additional compounds were prepared: octylmercaptomethylphosphonic acid, dodecylmercaptomethylphosphonic acid, cyclohexylmercaptomethylphosphonic acid, benzylmercaptomethylphosphonic acid, phenylmercaptomethylphosphonic acid, dibutyl decylmercaptomethylphosphonate, phenyldecyldercaptomethyl acid phosphonate, dithiobutyl dodecylmercaptomethylphosphonate, dibutyl phenylmercaptomethylphosphonate, phenyldecyldercaptomethyl acid phosphonate, dithiobutyl dodecylmercaptomethylphosphonate, dibutyl phenylmercaptomethylphosphonate, dithiooctyl cyclohexylmercaptomethylthiophosphonate, dioctylamine dodecylmercaptomethylphosphonate, dioctadecylamine phenylmercaptomethylphosphonate, tert-octadecylamine dodecylmercaptomethylphosphonate and mixtures thereof.

The additives of this invention are novel compounds. They are oil-soluble and can be used in amounts of from about 0.1% to about 25%, preferably from about 0.5% to about 5.0% by weight.

Mercaptomethylphosphono compounds of this invention are outstanding additives for various liquid hydrocarbon products, such as natural and synthetic hydrocarbon lubricating oils, greases, fuels (gasoline, kerosene, gas oil, burner fuel oil), asphalts, waxes, slushing oil, industrial oils, e.g., metal working and drawing oils, quenching oils, textile oils, hydraulic oils, dielectric compositions and other industrial oils. They are particularly outstanding when added in small amounts to lubricating oils and lubricating compositions to impart extreme pressure and anti-wear properties to such materials. Also, these additives are useful additives for gasoline, fuel oils, and other light oil products.

The following compositions are illustrative of the invention, the percentages being by weight, of the indicated additive or additives with the remainder being essentially the base.

| Composition A:                                                                          | Percent |    |
|-----------------------------------------------------------------------------------------|---------|----|
| Example I additive                                                                      | 2       |    |
| 1010 mineral oil                                                                        | Balance | 50 |
| Composition B:                                                                          |         |    |
| Example II additive                                                                     | 2       |    |
| 1010 mineral oil                                                                        | Balance |    |
| Composition C:                                                                          |         |    |
| Example III additive                                                                    | 2       | 55 |
| 1010 mineral oil                                                                        | Balance |    |
| Composition D:                                                                          |         |    |
| Example IV additive                                                                     | 2       |    |
| 1010 mineral oil                                                                        | Balance |    |
| Composition E:                                                                          |         |    |
| Example II additive                                                                     | 1       |    |
| SAE 30 mineral oil                                                                      | Balance |    |
| Composition F:                                                                          |         |    |
| Example I additive                                                                      | 2       |    |
| SAE 90 mineral oil                                                                      | Balance | 65 |
| Composition G:                                                                          |         |    |
| Example I additive                                                                      | 2       |    |
| Lauric acid                                                                             | 2       |    |
| SAE 90 mineral oil                                                                      | Balance | 70 |
| Composition H:                                                                          |         |    |
| Example I additive                                                                      | 5       |    |
| Ucon 50HB660 (polyethylene - propylene glycol having a SUS viscosity at 100° F. of 660) | Balance | 75 |

|   |                                |         |
|---|--------------------------------|---------|
| 4 | Composition I:                 |         |
|   | Example I additive             | 2       |
|   | Di-2-ethylhexyl sebacate       | Balance |
| 5 | Composition J:                 |         |
|   | Example I additive             | 1       |
|   | Leaded gasoline (3 cc. of TEL) | Balance |
|   | Composition K:                 |         |
|   | Example I additive             | 0.1     |
|   | Fuel oil (No. 2)               | Balance |

10 Compositions of this invention were evaluated for their extreme pressure properties on a Spur-Gear machine. The machine consists essentially of two geometrically similar pairs of gears connected by two parallel shafts. The gear pairs are placed in separate gear boxes, which also contain the supporting ball bearings. One of the shafts consists of two sections connected by a coupling. Loading is accomplished by locking one side of the coupling and applying torque to the other. The conditions of the test were:

15 Speed r.p.m. 3200  
Oil temperature °C. 100  
Oil flow-rate cc./scc. 10  
25 Load in increments 5 min. at each setting.

20 Results of the evaluations are given in Table I and for the purpose of comparison, the results obtained from the use of the base oil alone and with other known extreme 30 pressure compositions are also given.

Table I

| Composition:                                                            | Score load, lbs./in. |
|-------------------------------------------------------------------------|----------------------|
| A through I                                                             | 5,600                |
| 1010 mineral oil +2% C <sub>16</sub> alkenyl succinic acid              | 1,400                |
| 1010 mineral oil +2% malonic acid                                       | 2,800                |
| 1010 mineral oil +2% 3-hexadecyl adipic acid                            | 1,400                |
| 1010 mineral oil +2% dodecylmercapto succinic acid                      | 1,400                |
| 1010 mineral oil +10% glycerol monooleate                               | 1,800                |
| 1010 mineral oil +2% C <sub>13</sub> H <sub>27</sub> OH ("Oxo" process) | 600                  |
| 1010 mineral oil                                                        | 600                  |

35 The following compositions were also tested for stability in the Dornte Oxidation Test described in the Natural Petroleum News, September 17, 1941, pages 294-6 under the following conditions: 302° F., iron catalyst, mineral white oil base and additive amount in each example was about 1% by weight and the results are shown in Table II.

Table II

|    | Additive                                                                                                                                                                                                       | Induction Period (hrs.) |
|----|----------------------------------------------------------------------------------------------------------------------------------------------------------------------------------------------------------------|-------------------------|
| 60 | 1. n-decylmercaptomethylphosphonic acid.....                                                                                                                                                                   | 140                     |
| 65 | (n-C <sub>10</sub> H <sub>21</sub> -S-CH <sub>2</sub> -P=O(OH) <sub>2</sub> )<br>2. 2-ethylhexylmercaptomethylphosphonic acid.....                                                                             | 80                      |
| 70 | (CH <sub>3</sub> CH <sub>2</sub> CH <sub>2</sub> CH <sub>2</sub> CH-CH <sub>2</sub> -S-CH <sub>2</sub> -P=O(OH) <sub>2</sub> )<br>C <sub>2</sub> H <sub>5</sub><br>3. n-decylmercaptoethylphosphonic acid..... | 14                      |
| 75 | (n-C <sub>10</sub> H <sub>21</sub> -S-CH <sub>2</sub> CH <sub>2</sub> -P=O(OH) <sub>2</sub> )                                                                                                                  |                         |

The mercaptomethylphosphono compounds of this invention are useful also for providing superior load-carrying properties for lubricating oils which contain minor amounts of other agents, such as silicone anti-foaming agents, alkylphenol anti-oxidants, polyacrylate ester viscosity-index improvers, long chain fatty acids such as lauric and oleic acids, oiliness agents and the like.

I claim as my invention:

1. As a compound a  $C_{10-18}$  alkyl mercaptomethylphosphonic acid.
2. As a compound, decyl mercaptomethylphosphonic acid.

10

**References Cited by the Examiner**

**UNITED STATES PATENTS**

|             |       |                 |       |         |
|-------------|-------|-----------------|-------|---------|
| 2,535,174   | 12/50 | Tawney          | ----- | 260—461 |
| 2,793,225   | 5/57  | Scott           | ----- | 260—461 |
| 5 2,963,505 | 12/60 | Muhlmann et al. | ----- | 260—461 |

**OTHER REFERENCES**

Arbuzov et al.; "J. Gen. Chem. U.S.S.R." (English translation), vol. 27, pp. 2419—2421 (1957).

CHARLES B. PARKER, *Primary Examiner.*